

## UNITED STATES PATENT OFFICE

VANDERVEER VOORHEES, OF WHITING, INDIANA, ASSIGNOR TO STANDARD OIL COMPANY, OF WHITING, INDIANA, A CORPORATION OF INDIANA

## PICKLING METALS

No Drawing. Continuation of application Serial No. 121,279, filed July 8, 1926. This application filed January 18, 1928. Serial No. 247,746.

This invention relates to the acid pickling of metals, and particularly to the reduction of hydrogen evolution and loss of metals therein.

According to the present invention hydrogen evolution and excessive attack of the metal are substantially reduced or prevented in the cleaning of metals, particularly ferrous metals, by pickling in an acid bath consisting wholly or in part of acid derived from acid sludge from the sulfuric acid treatment of a petroleum oil which has been subjected to cracking temperatures. It is preferred to employ acid derived from sludge resulting from the treatment with sulfuric acid of oils cracked under pressure at temperatures which are usually in excess of 700° F. Acid from sludges derived from distillate products, such as cracked gasoline and kerosene are preferred. As a specific example it may be stated that good results are obtained with acid recovered from sludge resulting from the treatment of pressure distillate, produced, for example, by the Burton process at temperatures of 720-760° F. and pressures above 4 atmospheres, with sulfuric acid of about 66° Baumé, although other acid strengths may be employed if desired.

While the restraining effect with regard to metal attack is possessed by the pressure distillate sludge, to a high degree, a preliminary treatment is necessary in order to avoid several objections which arise in actual practice. For example, if such sludge is diluted to the extent necessary to produce a pickling bath of normal acid content there would be a tendency for asphaltic matters to precipitate upon the metal under treatment, thereby preventing effective pickling and causing imperfections in the finished metal when subjected to tinning or other subsequent operations. Another objection is that the sludge possesses a nauseating odor when raised to pickling temperature. Both these disadvantages can be substantially completely over-

come by diluting the sludge with water so as to bring its concentration of acid below 40%, for example, and subjecting the diluted sludge to boiling or steaming. In actual practice it is preferred to dilute the sludge first to a concentration of 35 to 40%  $H_2SO_4$ . A tarry substance separates as a result of this treatment, especially if the liquid is allowed to stand. Such substance is removed and the acid layer, preferably diluted further to about 25 to 30%  $H_2SO_4$  and further steamed. This treatment effectively drives off volatile odors. The resulting acid is a clear, brownish red liquid which may be diluted directly to a concentration suitable for the pickling operation or may be admixed with other acid and diluted. No tarry matter separates on further dilution and its odor is greatly improved. The deodorized strong acid is relatively inactive towards ferrous metals and may suitably be transported in steel tank cars to the places where it is to be diluted and used in pickling.

It must be understood that the invention is not limited to the use of an acid derived from a sludge from pressure distillate, since good results may be obtained with acid from sludges derived from other distillates and residues from the various known cracking processes.

According to the invention, the pickling bath may be of any suitable concentration and may be used at any suitable temperature. Ordinarily the initial concentration used is between 5 and 10% of sulfuric acid although higher concentration may be used. A suitable pickling temperature is between 160 and 180° F. As indicated above, the pickling bath may consist exclusively or in part only, of acid derived from the sludge from cracked petroleum products. Such acid appears to contain bodies which act catalytically and gives excellent results when only a small part of the bath consists of acid from the sludge. For example, the sludge

75

80

85

90

751

acid may constitute as little as 5% or less of the total acid content. Below are given results which express in milligrams per square inch the corrosion loss determined with strips of clean black iron when immersed for ten minutes at 180° F. to baths of 5%  $H_2SO_4$ , the acid constituted by various proportions of chemically pure and sludge acids.

| 10 | Proportion of acids | Corrosion loss<br>(mgms.<br>per square<br>inch) |
|----|---------------------|-------------------------------------------------|
| 15 | 100% pure acid      | 18.2                                            |
|    | 75% pure acid       |                                                 |
|    | 25% sludge acid     | 1.4                                             |
|    | 85% pure acid       |                                                 |
|    | 15% sludge acid     | 2.4                                             |
|    | 95% pure acid       |                                                 |
|    | 5% sludge acid      | 5.3                                             |

20 This application is a continuation of my prior application Serial No. 121,279, filed July 8, 1926.

I claim:

1. The method of acid pickling metals which comprises subjecting the metal to the action of a pickling bath containing acid and incorporating in said bath organic substances recovered from sludge derived from a cracked petroleum distillate soluble in dilute sulfuric acid, said organic substances being free from sludge substances soluble in strong sulfuric acid and not soluble in dilute sulfuric acid.

2. The method of acid pickling metals which comprises subjecting the metal to the action of an acid pickling bath and incorporating in said bath organic substances derived from the sludge from acid treatment of a pressure cracked distillate and soluble in dilute sulfuric acid, said organic substances being free from sludge substances soluble in strong sulfuric acid, and not soluble in dilute sulfuric acid.

3. The method of acid pickling metals which comprises subjecting the metal to the action of an acid pickling bath and incorporating in said bath a material recovered from petroleum acid sludge containing organic substances therefrom soluble in dilute sulfuric acid, said material being free from sludge substances soluble in strong sulfuric acid and not soluble in dilute sulfuric acid.

4. The method of acid pickling metals which comprises subjecting the metal to the action of an acid pickling bath and incorporating in said bath a material recovered from petroleum acid sludge consisting of sulfuric acid and such organic substances thereof as are soluble in dilute sulfuric acid, said material being free from sludge substances soluble in strong sulfuric acid and not soluble in dilute sulfuric acid.

5. The method of acid pickling metals which comprises subjecting the metal to the action of an acid pickling bath and incorpo-

rating therein a material recovered from petroleum acid sludge consisting of sulfuric acid and such organic substances as are soluble in dilute sulfuric acid and free from sludge substances soluble in strong sulfuric acid and not soluble in dilute sulfuric acid, the acid of such material constituting from 5 to 25% of the total acid in the bath.

6. The method of preparing a bath for pickling metals which comprises diluting acid sludge derived from a cracked petroleum oil with water, heating to cause separation of asphaltic matter and incorporating the acid and accompanying organic substances soluble therein in a metal pickling bath.

7. The method of producing a metal pickling bath which consists in diluting sludge from the sulfuric acid treatment of cracked distillate with water, heating to cause separation of asphaltic material and expel odors, removing the asphaltic material and embodying the acid and accompanying organic substances soluble therein in a pickling bath of suitable strength.

8. A solution for pickling iron or steel articles, comprising water and a material recovered from petroleum acid sludge consisting of sulfuric acid and such organic substances as are soluble in dilute sulfuric acid, said material being free from sludge substances soluble in strong sulfuric acid and not soluble in dilute sulfuric acid.

9. A solution for pickling iron or steel articles, comprising commercial sulfuric acid, water and a material recovered from petroleum acid sludge consisting of sulfuric acid and such organic substances as are soluble in dilute sulfuric acid, said material being free from sludge substances soluble in strong sulfuric acid and not soluble in dilute sulfuric acid.

10. A solution for pickling iron or steel articles containing as an ingredient a material recovered from petroleum acid sludge consisting of sulfuric acid and such organic substances as are soluble in dilute sulfuric acid, and free from sludge substances soluble in strong sulfuric acid and not soluble in dilute sulfuric acid.

11. A solution for pickling iron or steel articles containing as ingredients commercial sulfuric acid and a material recovered from petroleum acid sludge consisting of sulfuric acid and such organic substances as are soluble in dilute sulfuric acid, and free from sludge substances soluble in strong sulfuric acid and not soluble in dilute sulfuric acid.

12. A solution for pickling iron and steel articles containing as ingredients commercial sulfuric acid and a material recovered from petroleum acid sludge consisting of sulfuric acid and such organic substances as are soluble in dilute sulfuric acid and free from sludge substances soluble in strong sulfuric acid and not soluble in dilute sulfuric acid,

the proportion of said material being such that the acid content thereof constitutes not less than 5% of the total acid of the bath.

13. A solution for pickling iron and steel articles comprising water and a material recovered from acid sludge from the treatment of cracked petroleum distillate and consisting of sulfuric acid and such organic substances as are soluble in dilute sulfuric acid, said material being free from sludge substances soluble in strong sulfuric acid and insoluble in dilute sulfuric acid.

14. A solution for pickling iron or steel articles comprising commercial sulfuric acid, water and a material recovered from acid sludge from the treatment of cracked petroleum distillate and comprising organic substances therefrom soluble in dilute sulfuric acid, said material being free from sludge substances soluble in strong sulfuric acid and not soluble in dilute sulfuric acid.

15. A solution for pickling iron or steel articles comprising sulfuric acid, water and a material recovered from petroleum acid sludge and containing such organic substances thereof as are soluble in dilute sulfuric acid, said material being free from sludge substances soluble in strong sulfuric acid and not soluble in dilute sulfuric acid.

30 In testimony whereof I have hereunto set my hand this 4th day of January, 1928.

VANDERVEER VOORHEES.

35

40

45

50

55

60

65